

# UNITED STATES PATENT OFFICE.

CHAD H. HUMPHRIES, OF KEARNEY, NEW JERSEY, ASSIGNOR TO THE COMMERCIAL RESEARCH COMPANY, OF LONG ISLAND CITY, NEW YORK, A CORPORATION OF NEW YORK.

## METAL ARTICLE AND PROCESS OF MAKING SAME.

1,229,960.

Specification of Letters Patent. Patented June 12, 1917.

No Drawing.

Application filed September 28, 1914. Serial No. 863,897.

To all whom it may concern:

Be it known that I, CHAD H. HUMPHRIES, a subject of the King of Great Britain, residing at Kearney, in the county of Hudson 5 and State of New Jersey, U. S. A., have invented certain new and useful Improvements in Metal Articles and Processes of Making Same, of which the following is a specification.

10 This invention relates to metal articles and processes of making same; and it comprises an article of hard, dense metal composed mainly of tungsten group metal and containing in addition to the tungsten metal 15 a smaller percentage of an interpenetrating integralizing or alloying metal, such uniting metal being advantageously a metal of the class of nickel, cobalt, iron or the like, said dense metal having a surface with the unattactable permanent characteristics of a noble metal and said dense metal being of relatively high electrical conductivity; and it further comprises a method of producing such metallic material wherein the metals to 20 be united are first produced in the form of fine-grained powders, the grain size of the tungsten group metal being advantageously within certain limits and such limits being so correlated with later heating conditions 25 as to secure a definite degree of interpenetration of such metals in such later operations, the powders are mixed in the desired proportions, the mixture is heated in a plurality of temperature stages, with a pause at 30 each stage, until a metallic material is produced which is hard, dense, malleable and of relatively high electrical conductivity, such heating however not being carried far enough to produce a material of microscopic 35 cal (as distinguished from mechanical) homogeneity and of high ductility and such material is thereafter worked down to swaged or hammered material; all as more fully hereinafter set forth and as claimed.

40 While the product and the process of the present invention may be used for other purposes, I shall hereinafter describe more specifically the production of metallic material for use as contact points or elements for 45 electrical purposes. Ordinarily, these contact elements assume the form of a rivetlike element secured in an orificed holding member which may be a spring or the like; and usually they are not integral or a single piece 50 of metal but are composed of assembled bodies of different metals. The reason for this

assemblage is in the necessity for the union of different metallic qualities. For electrical purposes, naturally the contact making surface should be of non-oxidizing (or "noble") metal to insure quick and positive making and breaking of the circuit. Any film of oxid or impairment of the bright metallic surface militates against positive metallic contact. Further, the surface should 60 be of high melting metal and be relatively hard and permanent to avoid mechanical wear and electrical erosion. The body of the contact element must be mechanically strong and hard to secure it in permanent union 65 with the holding element; and for this purpose it is also highly desirable that it be of such character as to permit "striking up" or riveting in place. Conditions of use in modern electrical devices and machinery are frequently so severe as to require great strength 70 and rigid attachment in these contacts; a type of attachment best secured by a rivet union.

No single metallic material available at 80 present possesses all these qualities to a sufficient degree. Platinum possesses the noble surface, but it is relatively soft, even when alloyed with iridium, etc., and wears electrically and mechanically, while it is not 85 a strong metal. It is also an expensive material. Tungsten, as at present produced, while high melting and hard and strong oxidizes to some extent and moreover is not sufficiently workable to permit striking it up to 90 form a riveted union with a holding element.

In the present art therefore high grade contact elements are customarily made of two or more metals and are not made of a single piece of one metal. The best are 95 made by weld uniting a facing layer of platinum to a shank of nickel, the platinum giving the permanent surface and the nickel the strength.

I have found that I can produce a composite metallic material from which strong, noble-surfaced rivetable contact points can be made and which is also applicable to many other purposes requiring incorrodible acid proof strong metal, such as tooth pins, 100 commutator segments, anodes, jewelry, etc. To this end, I produce a material which though mainly tungsten contains another or integralizing metal bonding and qualifying the tungsten in a special way. This second metal is a metal of the iron class such as cobalt or iron. Nickel is much the best. 110

The proportion of tungsten in the completed material is best around 85 to 95 per cent. For some purposes it is advantageous to have some molybdenum. The present method may indeed be applied to the manufacture of composite molybdenum articles containing small proportions of tungsten or no tungsten. Molybdenum is a hard strong metal of much the same character as tungsten and although it oxidizes somewhat more easily the oxid volatilizes with comparative readiness and in situations where the oxids tend to form, as on hot contact points, it tends to disappear as readily. A small proportion, say 0.5 to 3 per cent. of molybdenum used with tungsten, makes a material of even more "noble" characteristics than the tungsten alone.

While tungsten is, by present methods, not readily worked to produce articles of the character here desired, I have found that by the present method I can make a material which is mainly tungsten and is hard, dense, conductive and sufficiently malleable for the present purposes. It possesses the valuable properties of tungsten as prepared by the best methods now in use and in an enhanced degree. This material while not ductile in the sense of being readily drawn down to wire, can be swaged and worked to produce bodies of compact metal suitable for contact points, tooth-pins, etc. When formed into a contact point it is sufficiently workable to allow heading up or riveting into place; something which cannot be done with the present grades of tungsten.

In preparing my material I use fine powdered tungsten of cryptocrystalline or semi-amorphous character. It is best that it be sufficiently fine to pass through a two hundred mesh sieve but not be completely impalpable or of "colloid" character. The best material for my purpose is of dark gray rather than light gray color, and is free of perceptible brownish spots or hue. The material may have a slight brownish cast but is best not distinctly brown. A coarser powder requires a longer heating period than the times hereinafter indicated and other modifications in conditions of operations; and I shall hereinafter refer more particularly to a powder of the indicated character. The tungsten is best not coarsely crystalline. It need not be perfectly pure, a certain amount of impurities indeed appearing to facilitate the operation in the specific method hereinafter described. It may be made by reduction from commercial tungstic oxid (or tungstic acid) by hydrogen. The commercial grade of tungstic acid is suitable. One oxid which I have used with advantage contains about 0.2 per cent. of alkalis and about the same amount of phosphoric acid. To make a suitable metal this crude oxid can be reduced by hy-

drogen in any suitable reduction furnace, care being taken that the temperature rises quite slowly during the operation and that the metal remains amorphous without becoming coarse and crystalline. The reduction is ordinarily not carried to the point of the complete disappearance of oxygen, a small amount of oxygen being left in the material.

With this tungsten I mix finely divided nickel or similar metal, which may be obtained by reduction in a similar manner. Nickel oxid or oxalate may be reduced at a low temperature. Reduction of oxid by hydrogen may be performed in any suitable type of apparatus. In reduction the temperature should not rise quickly enough to make the metal coarse grained. It should be as amorphous and fine grained as possible. A perceptible grain size is not here, as in the case of tungsten, desirable; the nickel should be completely impalpable. Metal produced from the oxalate is finer than that from the oxid. Reduction of the oxid by hydrogen may be performed around 300° C. Reduction is ordinarily interrupted at a point where some oxygen still remains; say not over 2 per cent. This reduction results in the formation of a velvety black and indefinitely fine powder of metallic nickel which is often pyrophoric. Therefore care should be taken in handling.

The two metals are very carefully mixed in the desired proportions. For making contact points and like purposes, a mixture of 85 per cent. to 95 per cent. tungsten and 15 to 5 per cent. nickel makes a useful material. A material of 6 to 8 per cent. is ordinarily employed in making contact points for general purposes. In obtaining such material a little more nickel is ordinarily used (say a few tenths per cent.) than is desired in the final material to allow for losses by volatilization. As to the amount of this allowance however much depends on the care with which the operation is carried out.

The mixed metals are next formed into bars or slabs in a steel mold by heavy hydraulic pressure. To facilitate this shaping a little temporary binder, such as a solution of camphor in ether, may be advantageously used. For example, a bar of square cross section one quarter inch on the side and 8 inches long may be made by heavily pressing about 85 grams of the described mixture. It is desirable in the present process with the specific procedure hereinafter indicated, to work with shaped bodies of about this order of magnitude. Other dimensions or shapes require some changes in the time and temperatures hereinafter set forth. The bar or "slug" is now sintered in a hydrogen atmosphere. During this operation it may rest on a nickel sup-

port. Heating, which may be by fire heat, should be gradual to prevent disruption by volatilization or carbonization of the binder, if a binder be used. The best temperature I have found is from 800° to 1100° C. and the treatment may be for about ten minutes. The slug is then allowed to cool in an atmosphere of hydrogen or other non-oxidizing atmosphere. After cooling it will be found to have changed from a dark to a light gray color and to present the appearance of a hard coked mass. It is not ductile and on the contrary it is exceedingly brittle, easily breaking into pieces. This sintered slug or billet is next heated in a plurality of temperature stages with a pause at each stage. Heating may now be effected by an electric current passed through the slug and should take place in an atmosphere containing hydrogen. The first heating should be to about 1200° C., the temperature being maintained as nearly at this point as practicable. The slug may be held at this temperature for about five minutes. One purpose of this operation is to cause an elimination of impurities contained in the tungsten and nickel. These impurities are alkalies, phosphoric acid, etc. Oxygen is also substantially removed. During this heating operation the impurities volatilize and form a sort of fog, giving a distinct tint to the flame if escaping hydrogen be ignited. About five minutes' heating at this temperature is ordinarily sufficient to cause the disappearance of most of the fog with the slug described. This heating may be called the purifying stage. The temperature is then again raised, this time to about 1400° C. This temperature should be maintained as nearly as practicable and it is best to conduct the operation with the aid of an optical or other high-temperature pyrometer. In this heating stage the mass shrinks considerably and traces of impurities are eliminated. Heating is in an atmosphere containing hydrogen. This heating stage may be called the shrinking stage and ordinarily requires about 5 minutes. The shrunk billet is now raised in temperature, this time to about 1600°. The exact temperature required will vary somewhat with the percentage of nickel in the mixture and other conditions. At this temperature nickel is freely fluid. Heating may be continued for about five minutes. This heating which may be called the integralizing stage has for its purpose union of the tungsten and nickel and the production of a hard, dense metal body which can be swaged. In this union the nickel and tungsten alloy and interpenetrate to a large extent.

In working with the nickel-tungsten mixture described, containing 6 to 8 per cent. nickel, the directions just given should be adhered to quite closely as regards tempera-

tures and times, since otherwise the results are not dependable and the final billets may be unworkable. With higher proportions of nickel the final temperature should be somewhat lowered. Too long a final heating or too fine or too coarse grained a tungsten give a non-swageable material, with the specific process now under description.

The material obtained after the integralizing stage upon cooling is not ductile in the sense in which the word is usually employed and it cannot be bent cold without causing fracture. Examined under the microscope it is seen to be fine grained and dense in texture. The billet of this material now may be swaged or rolled down to smaller size, becoming more compact, tenacious and hard with each working. Either hot or cold swaging may be used; and annealing may be resorted to.

In hot swaging, the finished slug may be reheated to 1200° to 1500° C., the temperature depending on the composition. With the material containing 6 to 8 per cent. nickel about 1400° is best. It is then taken to a high speed swaging machine giving, say, 5000 blows per minute and worked down, being reheated at intervals. As the operation progresses the temperature may drop and the speed of the swaging machine may be increased finally becoming, say, 7000 blows. In making contact elements, the reduction of the stated slug may be to a round body of, say, 0.16 to 0.125 inch. Pieces of this round body or rod of suitable length may next be given a shank by grinding or cutting. As the metal is quite hard this shank making operation may advantageously be effected by an emery or carborundum wheel. If the contact element is to be mounted in an orificed metal holding element, such as a spring, which is usually the case, the shank should be made to give a tight fit with the orifice. On assembling the contact element with the holding element, the protruding end of the shank may be upset or headed with a prick punch, giving a rivet head.

A wafer or disk of the metal may be welded to a shank of another metal to give a composite contact element (like those made with platinum). So used my metal offers the same mechanical and electrical advantages. But I regard the integral or one-piece contact as much better.

The slug may be cold swaged if desired, being sufficiently malleable for this purpose. It should be occasionally annealed, say after each 3 or 5 passes, or after a reduction of, say, 0.025 inch in diameter.

Metal produced as described is sufficiently malleable to permit swaging as described; and also to permit heading up to give a firm, permanent and secure rivetlike union

70

75

80

85

90

95

100

105

110

115

120

125

130

with a holding element. In so heading up the fiber of the metal permits the formation of the head.

A metal with 6 to 8 per cent. nickel and the residue tungsten has a melting point higher than that of platinum and suffers little erosion or wear when used for electrical purposes. It is also much harder than platinum or platinum-iridium alloys and wears much better. It does not have the tendency to film over with a skin of oxid which is displayed by pure tungsten. It is exceedingly acid-resistant making it particularly suitable for tooth-pins, anodes, etc.

In the foregoing method, iron or cobalt, may be used in lieu of the nickel either in whole or in part, but I find nickel or its alloys to be well adapted. With these other metals the indicated temperatures, etc., must be somewhat modified. The oxid of the particular metal to be used is reduced in the manner indicated for nickel oxid. In lieu of the tungsten may be substituted molybdenum. But for general purposes I find that the metal containing tungsten and nickel, with or without some molybdenum, is best suited.

It will be noted that in the described method an intimate mixture of fine-grained tungsten powder with a small amount of another pulveriform metal of lower melting point (best, nickel) is heated progressively in discrete temperature stages, with the final heating at a temperature at which the binder metal is capable of being freely liquid but far below that at which the tungsten particles themselves will melt. This temperature is also far below that at which an alloy of the two metals in the chosen proportions will liquefy. This heating is interrupted at a time when the metallic mass becomes unified or integralized by interpenetration of the two metals sufficiently to allow the mass to be worked down. Continuance of the mutual action of the tungsten and bonding metal upon each other results in the production of a material which is more in the nature of a true alloy and which has properties of a type not here desired. The present material is more in the nature of a bonded body of tungsten.

Owing to the fine grained, dense, non-porous character of the final product produced after swaging down, and the intimate manner in which the interpenetrating metals are united, its electrical conductivity is relatively high as compared with the fibrous, ductile, tungsten materials produced for incandescent lamp filaments. In a filament, naturally, the object is to secure a good resistance, while in making contact points conductivity is an advantage.

After the described operations the material produced is of such character as to permit machining and cutting but by a heat

treatment, which may be applied after shaping, it can be made hard enough to resist all ordinary cutting tools. In this treatment it may be raised to, say, 1600° C. and then suddenly cooled by immersion in water. 70

What I claim is:—

1. As a new material, a hard, dense relatively conductive, mechanically homogeneous fine-grained metallic mass mainly composed of particles of a metal of the tungsten class but also containing another and bonding metal of lower melting point, said mass being substantially non-ductile but malleable to an extent which will permit swaging hot or cold. 75

2. As a new material, a hard, dense relatively conductive, mechanically homogeneous fine-grained metallic mass mainly composed of particles of tungsten but also containing another and bonding metal of lower melting point, said mass being substantially non-ductile but malleable to an extent which will permit swaging hot or cold. 80

3. As a new material, a hard, dense relatively conductive, mechanically homogeneous fine-grained metallic mass mainly composed of particles of a metal of the tungsten class but also containing a little nickel as a bonding material, said mass being substantially non-ductile but malleable to an extent which will permit swaging hot or cold. 90

4. As a new material, a hard, dense relatively conductive, mechanically homogeneous fine-grained metallic mass mainly composed of particles of tungsten but also containing a little nickel as a bonding material, said mass being substantially non-ductile but malleable to an extent which will permit swaging hot or cold. 100

5. As a new material, a metallic mass composed of fine-grained tungsten with its particles bonded and united by a relatively small amount of lower melting metal in a dense hard malleable but substantially non-ductile body. 110

6. As a new material, a metallic mass composed of particles of fine-grained tungsten bonded and united by a relatively small amount of nickel in a dense hard malleable but substantially non-ductile body. 115

7. In the manufacture of tungsten materials, the process which comprises mixing a finely grained metal of the tungsten class with another metal of lower melting point, heating the mixture to a temperature at which said other metal is freely fluid and holding at this temperature sufficiently long to permit a limited degree of interpenetration without complete alloying of the two metals. 120

8. In the manufacture of tungsten materials, the process which comprises mixing finely grained tungsten with another metal 125

- of lower melting point, heating the mixture to a temperature at which said other metal is freely fluid and holding at this temperature sufficiently long to permit a limited degree of interpenetration without complete alloying of the two metals. 5
9. In the manufacture of tungsten materials, the process which comprises mixing a finely grained metal of the tungsten class with nickel, heating the mixture to a temperature at which said nickel is freely fluid and holding at this temperature sufficiently long to permit a limited degree of interpenetration without complete alloying of the two metals. 10
10. In the manufacture of tungsten materials, the process which comprises mixing finely grained tungsten with nickel, heating the mixture to a temperature at which said nickel is freely fluid and holding at this temperature sufficiently long to permit a limited degree of interpenetration without complete alloying of the two metals. 15
11. In the production of hard, dense tungsten materials, the process which comprises intimately mixing fine-grained tungsten with a pulveriform metal of the iron class and heating the mixture at a temperature at which said metal is freely liquid but below the melting point of tungsten and below the melting point of an alloy containing tungsten and said other metal in the same proportion, said heating being interrupted when the mass becomes malleable enough to 20 swage and before any substantial alloying has taken place. 25
12. In the production of hard, dense tungsten materials, the process which comprises intimately mixing fine-grained tungsten with pulveriform nickel and heating the mixture at a temperature at which said nickel is freely liquid and below the melting point of tungsten and below the melting point of an alloy containing tungsten and said nickel in the same proportion, said heating being interrupted when the mass becomes malleable enough to 30 swage. 35
13. In the manufacture of composite tungsten articles, the process which comprises mixing fine-grained tungsten with a minor amount of a lower melting pulveriform metal of the iron class, heating the mass sufficiently to sinter it, continuing the heating after the sintering and elevating the temperature sufficiently to eliminate impurities, and then elevating the temperature to a point above the melting point of the other metal, heating at this temperature being continued until the mass becomes malleable 40 enough to swage. 45
14. In the manufacture of composite tungsten articles, the process which comprises mixing fine-grained tungsten with a minor amount of pulveriform nickel, heating the mass sufficiently to sinter it, continuing the heating after the sintering and elevating the temperature sufficiently to eliminate impurities, and then elevating the temperature to a point above the melting point of the other metal, heating at this temperature being continued until the mass becomes malleable enough to swage. 50
15. In the manufacture of composite tungsten articles, the process which comprises mixing fine-grained tungsten with a pulveriform bonding metal, heating the mixture to a temperature at which it will sinter, further heating the mixture at about 1200° C. until contained impurities are substantially removed and elevating the temperature to a point at which the bonding metal is freely fluid, the last stated heating being continued until the mass becomes malleable enough to 55 swage. 60
16. In the manufacture of composite tungsten articles, the process which comprises mixing fine-grained tungsten with pulveriform nickel, heating the mixture to a temperature at which it will sinter, further heating the mixture at about 1200° C. until contained impurities are substantially removed and finally elevating the temperature to about 1600° C., this temperature being maintained until the mass becomes malleable enough to 65 swage. 70
17. In the manufacture of composite tungsten articles, the process which comprises sintering an intimate mixture of fine-grained tungsten with a minor amount of a lower melting bonding metal, heating the sintered mass to a temperature at which volatile impurities will be dispelled, heating the purified mass to a higher temperature to shrink it, and finally heating the shrunk mass to a temperature above the melting point of the bonding metal, the heating being continued until the mass becomes malleable 80 enough to swage. 85
18. In the manufacture of composite tungsten articles, the process which comprises sintering an intimate mixture of fine-grained tungsten with a minor amount of nickel, heating the sintered mass to a temperature at which volatile impurities will be dispelled, heating the purified mass to a higher temperature to shrink it, and finally heating the shrunk mass to a temperature about 90 1600° C., the heating being continued until the mass becomes malleable enough to 95 swage. 100
19. In the manufacture of composite tungsten articles, the process which comprises heating a sintered intimate mixture of fine-grained tungsten and fine-grained nickel to a temperature at which the nickel is freely fluid, heating at this temperature being continued until a sufficient degree of interpenetration of the metals is secured to make the mass malleable enough to 105 swage. 110
20. In the manufacture of composite tungsten articles, the process which comprises 115

- sintering an intimate mixture of fine-grained tungsten and fine-grained nickel, purifying the sintered mass by elevating the temperature sufficiently to volatilize impurities, after 5 maintaining at such volatilization temperature for a sufficient length of time heating to a temperature at which the mass will shrink and become compact, after maintaining the heat at such shrinking temperature 10 for a sufficient length of time elevating the temperature to around 1600° C. and maintaining the temperature at this point until the mass becomes malleable enough to swage.
21. In the manufacture of composite tungsten articles, the process which comprises 15 producing an intimate mixture of fine-

grained tungsten and fine-grained nickel, both such tungsten and such nickel containing a small proportion of residual oxid, sintering the mass, heating to a temperature 20 at which impurities will volatilize, heating to a temperature at which the mass will shrink and finally heating to about 1600° C. until the mass becomes malleable enough to swage.

25  
In testimony whereof, I affix my signature in the presence of two subscribing witnesses.

CHAD H. HUMPHRIES.

Witnesses:

M. J. MACDONALD,  
GEORGE P. SCHOLE.